

Jan. 6, 1925.

1,521,881

J. H. HASTE

PHOTOGRAPHIC FILM WITH LAMINATED SUPPORT HAVING INCREASED FLEXIBILITY

Filed Dec. 26, 1922



INVENTOR  
James H. Haste,  
BY R. L. Stinchfield

ATTORNEY

## UNITED STATES PATENT OFFICE.

JAMES H. HASTE, OF ROCHESTER, NEW YORK, ASSIGNOR TO EASTMAN KODAK COMPANY, OF ROCHESTER, NEW YORK, A CORPORATION OF NEW YORK.

## PHOTOGRAPHIC FILM WITH LAMINATED SUPPORT HAVING INCREASED FLEXIBILITY.

Application filed December 26, 1922. Serial No. 609,124.

To all whom it may concern:

Be it known that I, JAMES H. HASTE, a citizen of the United States of America, residing at Rochester, in the county of Monroe 5 and State of New York, have invented certain new and useful Improvements in Photographic Films with Laminated Supports Having Increased Flexibility, of which the following is a full, clear, and 10 exact specification.

This invention relates to photographic film, the base of which is laminated. The principal object of the invention is to so construct the film that the flexibility thereof will be increased both as regards degree and permanence. Other objects will hereinafter appear.

In the accompanying drawing the single figure shows in diagrammatic cross section 20 upon an exaggerated scale a film embodying one form of my invention.

While endeavoring to increase the flexibility of photographic films both as regards the degree of flexibility and the time during 25 which the flexibility will last, I have discovered that the desired result may be obtained by providing a laminated support, the layers of which are interunited throughout their entire adjacent faces, the material 30 present in the zone or layer of interunion containing a greater amount of flexibility-inducing material than the main bodies of the supporting layers or laminations. For these laminations I prefer to use compositions 35 consisting chiefly of cellulose addition compounds, such as cellulose nitrate, cellulose acetate and cellulose ether. The layers of these substances may contain the usual flexibility-inducing substances, such as butyl 40 or amyl alcohol, butyl or amyl acetate, monochlornaphthalene, tricresyl phosphate, castor oil, ethyl propionate, ethyl butyrate. This list is intended merely to be illustrative.

45 The flexibility-inducing substances cannot be present in too large an amount in the laminations without impairing other qualities of the film, such as strength, hardness and the like. The fact has been established, 50 however, that if a cement be used for uniting the laminations containing considerable amounts of flexibility-inducing material, the flexibility of the film will be surprisingly

increased above what might be expected when the relative thinness of the interuniting zone is considered. The flexibility-inducing material in the cement is added to and blended with the composition in the zone which already contains the normal amount of flexibility-inducing material. 60 Consequently a reserve or high percentage of the latter is built up in said zone. In other words, at the zone there is an intermingling of the compositions composing the laminations with the cementing material. 65 The volatile ingredients of the cement rapidly work outward through the bodies of the layers, but the relatively high-boiling flexibility-inducing substances remain in the form of a reserve in the zone of interunion where they continue to function 70 considerably longer than the normal amounts of flexibility-inducing substances do in conventional films of ordinary composition and structure. 75

Referring to the drawing in which one embodiment of my invention is shown by way of illustration, 1 indicates the photographically sensitive layer of any usual or preferred form,—say a layer of gelatino 80 silver haloid emulsion. The supporting layers of cellulosic addition compounds are indicated at 2. In the preferred form of my invention these layers are composed of nitro-cellulose and flexibility-inducing substances such as butyl alcohol and small amounts of castor oil or camphor. These layers are preferably formed as separate sheets and then cemented together in any known or preferred process or apparatus 85 for laminating such sheets by means of a cement containing a reserve of flexibility-inducing material. One suitable cement, by way of illustration, is acetone 20 parts, methyl alcohol 20 parts, methyl acetate 40 90 parts, butyl acetate 19 parts, nitrocellulose a trace, say 1 part, and a flexibility-inducing material such as monochlornaphthalene, tricresyl phosphate or butyl alcohol, castor oil, etc., from 2 to 10 parts. No matter 100 what the percentage of flexibility-inducing material be in the compositions of the laminations, the zone of interunion formed by the blending action of the cement will contain in addition the flexibility-inducing 105 material introduced by the cement. Thus a

reserve is created which has the surprising effects described above.

Having thus described my invention, what I claim as new and desire to secure by Letters Patent is:

1. As an article of manufacture, a photographic film comprising a photographically sensitive layer and a laminated, flexible, transparent, support therefor, said support including a plurality of layers of a cellulosic addition compound, mixed with flexibility-inducing material, said layers being interunited throughout their entire adjacent faces, this zone of interunion being thinner than said layers and containing cellulosic compound from said layers and also containing a greater proportion of flexibility-
- 10
- 15

inducing material than said layers, thereby embodying a reserve of said material.

2. As an article of manufacture, a photographic film comprising a photographically sensitive layer and laminated, flexible, transparent, support therefor, said support including two layers of nitrocellulose composition united throughout their entire adjacent faces, this zone of interunion being thinner than said layers and containing nitrocellulose from said layers and also containing a reserve of flexibility-inducing material of low volatility.
- 20
- 25
- 30

Signed at Rochester, New York, this 16th day of December, 1922.

JAMES H. HASTE.